

## UNITED STATES PATENT OFFICE

JOSEPH PIERRE LEEMANS, OF HOBOKEN-LEZ-ANVERS, BELGIUM, ASSIGNOR TO SOCIETE GENERALE METALLURGIQUE DE HOBOKEN, OF HOBOKEN-LEZ-ANVERS, BELGIUM

## REFINING OF COPPER

No Drawing. Application filed June 22, 1931, Serial No. 546,155, and in Germany January 3, 1931.

This invention relates to a process for the refining of black copper, with a view to obtaining anodes for electrolytic refining, and applies more particularly to very impure black copper, containing for instance from 80 to 95% of copper, the impurities being mainly metals of the iron group, such as iron, cobalt and nickel.

Hitherto, the black copper was charged in a flame oven, called "anode furnace" having for its function to smelt the copper, to effect the oxidation of the impurities by concentrating the latter in a slag which floats at the surface of the molten bath, to reduce by poling the oxide of copper which has been formed during the previous operation, and lastly to cast the refined copper in the form of anodes with a view to electrolytic treatment.

During the operation of refining in the anode furnace, a more or less important amount of slag is produced, according to the percentage of impurities contained by the black copper.

This slag may contain up to 35% of copper or more, partly in metallic form, partly in the form of oxides or silicates.

The recovery of the copper contained in the slags obtained by the refining operation was hitherto effected by melting the slag in the presence of coke and of fluxes. This operation is carried apart from the smelting of black copper and requires a large consumption of fuel.

It has been ascertained that by smelting the slag obtained from the refining of black copper in the presence of a suitable amount of black copper, the elimination of the copper contained in the said slag is effected by the impurities, namely iron and ferrous metals, contained in the black copper. It follows that the black copper acts by its impurities as a precipitating agent for the copper contained by the slag; conversely the latter acts as a purification agent for the black copper.

This action is due to the fact that the copper contained by the slags obtained in the refining operation, is partly in oxide form.

During the smelting operation the oxide of copper reacts with the impurities, namely with the iron and ferrous metals contained in the black copper, and produces their scoriaction. An important advantage of the simultaneous smelting operation is that it is exothermal. It therefore supplies the smelting of a mixture of black copper and slag from the refining operation, with a portion of the heat which is necessary for the smelting, thus saving an important amount of fuel.

The above facts have permitted to bring into effect a new process for the refining of black copper, more particularly with a view to obtaining anodes for the electrolytic refining.

According to a characteristic feature of the present invention, the black copper to be treated is subjected to simultaneous smelting with the slag containing copper in oxide form, obtained from the subsequent refining operations. The smelting is preferably carried out in a shaft furnace of the water-jacket type. The copper thus treated is separated and is further treated in another furnace until obtaining anode copper.

By the said smelting a complete or partial purification of the black copper will be obtained according to the ratio black copper-slag which it has been possible to produce.

In the case of a normal black copper, that is containing a high percentage of copper (for instance 98 per cent), the copper obtained by the smelting with slag which contains oxide of copper, is generally sufficiently purified that it does not require any other subsequent oxidation than that necessary for the elimination of impurities other than those formed by metals of the ferrous group. This operation is then carried out in an anode furnace.

When however the black copper is very impure (containing for instance 80 to 95 per cent of copper), it is possible that the amount of slag available from the refining operation is not sufficient for obtaining a complete elimination of the metals of the ferrous group, and it is necessary to con-

tinue in another furnace the refining operation which was commenced by the smelting in the water-jacket furnace.

In this case, the purifying operation in the water-jacket furnace is followed by a blasting of the partially purified copper obtained in the water-jacket furnace, inside a tilting cylindrical furnace, or converter, provided with nozzles for the blast and with a device permitting to heat the apparatus. The blasted copper is afterwards removed into a reverberatory furnace where it is subjected to the operation of poling, and is cast in the form of anodes, or the poling may be carried out in the tilting furnace itself and the copper obtained may be cast direct.

The treatment of very impure black copper is thus effected in various apparatus, each adapted to the various treatments to which the black copper is to be subjected.

In this process the slag obtained in the converter and which contains copper in oxide form, is re-treated at the same time as black copper, inside the water-jacket furnace. The major part of the nickel remains alloyed with the copper, whilst the

major part of the cobalt passes into the slag, and the latter can be treated direct for obtaining a rich cobalt alloy.

I claim:

1. A process for the preliminary refining of black copper containing a high percentage of impurities of the iron group consisting of iron, nickel and cobalt, comprising the smelting of the black copper inside a shaft furnace together with slag containing copper oxides and without the addition of lime, so as to concentrate on the one side the copper, and on the other side the said impurities inside the shaft furnace, as set forth. 70

2. A process for the refining of black copper containing a high percentage of impurities of the iron group consisting of iron, nickel and cobalt, comprising the smelting of the black copper inside a shaft furnace together with slag containing copper oxides and without the addition of lime, and the further refining of the metal obtained in the shaft furnace by blasting and poling, so as to obtain anode copper, as set forth. 75

JOSEPH PIERRE LEEMANS.

30

95

35

100

40

105

45

110

50

115

55

120

60

125

65

130